

## UNITED STATES PATENT OFFICE.

MARION H. MERRISS, OF WESTBURY, NEW YORK, ASSIGNOR TO NICHOLS COPPER COMPANY, OF NEW YORK, N. Y., A CORPORATION OF NEW YORK.

## CONVERSION OF CUPROUS MATERIALS.

No Drawing.

Application filed August 1, 1925. Serial No. 47,638.

To all whom it may concern:

Be it known that I, MARION H. MERRISS, a citizen of the United States, and resident of Westbury, Long Island, Nassau County, 5 State of New York, have invented certain new and useful Improvements in the Conversion of Cuprous Materials, of which the following is a specification.

This invention relates to methods or 10 processes for converting black copper or like materials into blister copper.

"Black copper" as commonly known is a product of the direct smelting of oxidized ores or residues in a blast furnace with a reducing atmosphere. The copper of such material normally amounts to approximately 15 from 74 per cent to 94 per cent with comparatively large percentages of lead, zinc, tin, iron and other impurities. An 20 analysis of two typical samples of black copper such as may be used with this process reveals the following percentage compositions—

| 25 | Copper.             | Ar-senic.         | Anti-mony.        | Lead.            | Tin.              | Zinc.             | Nickel and cobalt. | Iron.             |
|----|---------------------|-------------------|-------------------|------------------|-------------------|-------------------|--------------------|-------------------|
| 30 | %<br>83.61<br>78.75 | %<br>.039<br>.031 | %<br>.191<br>.198 | %<br>.67<br>5.07 | %<br>3.80<br>6.74 | %<br>3.12<br>4.50 | %<br>.38<br>.52    | %<br>4.37<br>3.28 |

Also small and generally substantially negligible quantities of sulphur, aluminum oxide, silver and gold are often present.

35 The process of this invention is also applicable to the reclamation of the copper from brass, bronze and other materials having a composition somewhat analogous to that of black copper, and the conversion of 40 such materials by this process is intended to fall within the scope of the invention disclosed and claimed in this application.

It is an aim of this invention to provide a process for converting black copper or the 45 like materials to blister copper independently of other metallurgical operations. Furthermore, it is also an object of this invention to accomplish such conversion by a process which is economical and convenient 50 to practice in connection with a wide variety of ores or other material and the results of which are very dependable.

Heretofore in most instances black copper

or like materials have been economically converted to blister copper only by utilizing 55 the excess heat produced in the bessemerizing process of converting copper matte (a mixture of iron sulphide and copper sulphide) or white metal (copper sulphide). The conversion of copper matte is carried 60 out without the application of external heat since the process is in fact exothermic. There are certain classes of materials available in large quantities which may be added 65 during the conversion of the copper matte to blister copper, such materials thus being also simultaneously smelted into the form of blister copper. Among such materials may be included black copper and brass materials.

70 However, the combining of the treatment of copper matte with the conversion of black copper often involves serious difficulties. Although the causes of such difficulties are not well understood, it is believed that some 75 of the iron present in large quantities in the matte combines with the zinc of the black copper or brass to form substantial quantities of zinc ferrite, an extremely infusible material. This material settles out and 80 coats the interior of the converter, particularly the nose thereof, and eventually renders the opening too small for efficient use. It is also thought possible that an infusible 85 incrustation comprising a compound of magnetite, zinc oxide and zinc silicate may be formed. In any event undesirable incrustations are formed upon the interior of the converter which reduce the available space 90 therein and limit the amount of cold material which may be introduced.

The above described difficulties together 95 with the fact that there is often a supply of brass or black copper in excess of that which may be treated with copper matte, renders it desirable to provide a process for converting such material to blister copper independently of the copper matte conversion. I have discovered that if the black copper 100 or the like metals are given a preliminary or initial heating to start the operation, sufficient heat can be generated in a converter, by the oxidation of the impurities contained in such metals to enable the conversion of such cuprous metals to blister copper, and 105 according to this invention black copper and

the like cuprous metals are converted by subjecting them to an initial or preliminary heating operation sufficient to initiate oxidation of the impurities upon blowing an oxidizing fluid into the mass, and then converting the copper by blowing an oxidizing fluid, such for example as air, into the mass and relying substantially upon the heat generated by the oxidation of the impurities of the mass to effect the conversion.

The invention consists in the process and steps of the process which are herein described according to the preferred manner of practicing the same, and the invention will be particularly pointed out in the appended claims.

One example of the manner in which the invention may be satisfactorily carried out is as follows: The black copper or like material as above described is mixed with from 10 to 25 per cent of coke in a small red hot converter. The coke comprises fuel for initiating the process, such fuel being ignited by the hot converter, the heated condition of which also assists in starting the process. A quantity of wood may also be included for more rapidly igniting the coke and melting the charge.

After the converter is filled with this mixture, the air blower may be turned on with approximately four pounds of pressure for a period of from 15 to 20 minutes. During this time, the converter may be in a position with the flue disconnected. When the copper material starts to melt and the conversion reaction sets in, fumes will appear at the opening of the converter. The charge within the converter will have settled considerably by this time so that additional material may be introduced into the top thereof. Thereafter, the converter may be turned back upon its tuyères with its opening in a position to discharge fumes through the flue. For the next 10 or 15 minutes the blower should be adjusted to give a pressure of  $5\frac{1}{2}$  to 6 pounds. At the end of this period the pressure may be increased and maintained at the full normal working pressure of approximately 9 pounds during a period of about one hour, at which time the charge is brought to the finished condition of blister copper.

In carrying out the above described process for seven similar successive charges in the converter the total amounts of material introduced were as follows:

|                     | Pounds. |
|---------------------|---------|
| Black copper blocks | 14,946  |
| Black copper ingots | 7,913   |
| Light brick brass   | 21,650  |
| Oily brass turnings | 51,000  |
| Coke                | 14,000  |

It is found that the materials introduced in the relative proportions as above, give

very satisfactory results both as to quality of the blister copper formed and as to its cost as produced by the process. During the 7 charges above referred to, the coke consumed amounted to approximately 12.9% of the total weight of the charges. It will be understood that more or less coke may be used depending upon the character of the ore or brass being treated. For example if a larger proportion of oily brass turnings were used the amount of fuel necessary would be less in view of the fuel value of the oil.

The converter and blower equipment used may be of the type ordinarily used in the conversion of copper matte by the bessemerizing process.

The impurities which do not pass off as gaseous oxides form a slag which is preferably rendered liquid by suitable fluxing constituents, so that it can from time to time be skimmed from the surface or poured off. Suitable fluxing constituents are well known in the art and the particular materials used for such purposes will depend upon the nature of the impurities in the ore being treated. Irony material may be used to flux the coke ash and silicious materials will serve to flux any iron oxide which may be formed, since the silicate unites with the oxidized iron to form a liquid ferro-silicate.

As above indicated the materials most suitable for treatment by this process are black copper, brass or bronze or other copper bearing materials, which should preferably be in heavy pieces so that it may be handled cheaply and expeditiously and introduced into the converter in large quantities by weight within the limited space available. Brass or bronze borings and turnings, and fuse parts are suitable for the process. Lighter brass or other materials may also be used, although if their volume is great in proportion to their weight it becomes difficult to charge the converter at an economical rate.

It will be understood that the process may be started by using heat from sources other than by mixing fuel with the charge, for example, external sources of heat may be applied. Various fuels other than coke may also be used, if desired, or in certain instances it may be preferable to introduce the copper bearing material in the molten form, whether fuel or the various methods of initial extraneous firing are used. I have found that once the process is initiated, under most conditions there is sufficient heat given off by the oxidation of the impurities to be formed in these materials, to continue and complete the conversion of the copper content to blister copper. The heat produced by the oxidation of lead, zinc, carbon, tin or other impurities having a greater affinity for oxygen than copper, is thus economical.

ly used in carrying on the process once it has been started.

After the first charge in the converter has been converted to blister copper, the 5 process may be continued by a form of fractional blowing, that is, a portion of the molten blister copper may be retained in the converter as a heat reservoir. More of the 10 cold or partially warmed material with or without fuel may then be added and the resultant mixture blown to blister copper again, thereafter an additional 35 per cent, 50 per cent or 60 per cent of the product, as desired, may be removed and the operation 15 repeated. In this manner, the process of the invention may be carried out continuously with the use of very little fuel.

While I have described my invention according to the preferred embodiment of the 20 same it will be obvious to those skilled in the art, after understanding my invention, that various alterations, modifications and substitutions may be made without departing from the scope of the invention, and I aim 25 in the appended claims to cover all such modifications.

What is claimed as new and is desired to be secured by Letters Patent is:

1. The method of treating black copper 30 or the like materials embodying impurities which are largely in metallic form to obtain blister copper directly therefrom, which comprises preliminarily heating the mass of black copper or the like until it is at least 35 partially melted, then blowing air therethrough, controlling the quantity and pressure of the air to effect rapid oxidation of the impurities, and relying substantially upon the heat produced by such oxidation 40 for producing blister copper from the mass.

2. The method of obtaining blister copper directly by treatment of black copper or the like materials embodying impurities which are largely in metallic form and a 45 substantial portion of which form gaseous oxides of the metals, which method comprises preliminarily heating the mass of black copper or the like until it is at least partially melted, then blowing air therethrough in such quantity and at such pressure that rapid oxidation of the impurities is effected, relying substantially upon the heat produced by oxidation of the metallic impurities for producing blister copper 50 from the mass, and removing the resulting metallic oxides from the mass as gases and in slag.

3. The method of obtaining blister copper directly by treatment of black copper 60 containing impurities consisting of metals which form gaseous oxides and less than in the neighborhood of 10% of iron, which method comprises preliminarily heating the mass of black copper or the like until it is 65 at least partially melted, then blowing air

therethrough in such quantity and at such pressure that rapid oxidation of the impurities is effected, relying substantially upon the heat produced by oxidation of the metallic impurities for producing blister copper 70 from the mass, and removing the resulting iron oxide in slag and the other metallic oxides as gases.

4. The method of converting black copper or the like to blister copper by a bessemerizing process which comprises initiating the conversion process by mixing and burning approximately from 10% to 25% of carboniferous fuel with the black copper in a converter, and thereafter continuing the 80 process to a conclusion by utilizing the heat resulting from oxidation of impurities in the black copper having a greater affinity for oxygen than copper.

5. The method of converting into blister 85 copper various materials containing high percentages of copper and metallic impurities such as lead, zinc, tin, iron, etc. which comprises relying substantially solely upon the heat from oxidation of the said metallic 90 impurities and controlling such heat by an air blast to maintain the reaction temperature necessary for the conversion.

6. The method of converting black copper 95 or like materials to blister copper which comprises charging a hot converter with a mixture of the materials with sufficient fuel to initiate the conversion process, then introducing a gentle air blast, increasing and continuing the blast and utilizing the heat 100 from oxidation of the impurities in the mixture to continue and complete the conversion of the copper content in the charge to blister copper, and removing the slag 105 formed during the process.

7. The method of converting black copper 110 or like materials to blister copper which comprises charging a red hot converter with a mixture of the material in heavy pieces with sufficient coke as fuel to initiate the conversion process and fluxing constituents to liquidize the slag formed, then introducing a gentle air blast, thereafter increasing the air blast to full normal pressure, continuing the blast and utilizing the heat from 115 oxidation of the impurities in the mixture to continue and complete the conversion of the copper content to blister copper, and removing the slag formed during the process 120 by rabbling while the copper is still hot.

8. The method of converting black copper 125 or like materials to blister copper which comprises charging a red hot converter with a mixture of the material in heavy pieces with sufficient coke as fuel to initiate the conversion process and fluxing constituents to liquidize the slag formed, then introducing a gentle air blast, thereafter increasing the air blast to full normal pressure, and continuing the blast and utilizing the heat 130

from oxidation of the impurities in the mixture to continue and complete the conversion of the copper content to blister copper.

9. The method of forming blister copper from black copper or the like materials embodying impurities which are almost wholly metallic which comprises melting the material in a converter with fluxing constituents to liquidize the slag formed, introducing 10 into the converter a gentle air blast, and increasing and continuing the blast and utilizing the heat from oxidation of the metallic impurities in the mixture to continue and complete the conversion of the copper content to blister copper.

10. The method of converting black copper or like materials to blister copper which comprises charging a red hot converter with a mixture of the black copper in heavy 20 pieces with from 10% to 25% of carboniferous fuel to initiate the conversion process, then introducing a gentle air blast, thereafter increasing the air blast to full normal pressure continuing the blast and utilizing 25 the heat from oxidation of the impurities in the mixture to continue and complete the conversion of the copper content to blister copper.

11. The method of converting into blister 30 copper various materials containing high percentages of copper and impurities such

as lead, zinc, tin, iron, etc., which comprises charging a red hot converter with a mixture of the material in heavy pieces with sufficient coke as fuel to initiate the conversion 35 process, introducing a gentle air blast, thereafter increasing the air blast to full normal pressure, continuing the blast and utilizing the heat from oxidation of the impurities in the mixture to continue and complete the 40 conversion of the copper content to blister copper, and removing the slag formed during the process by rabbling while the copper is still hot.

12. The method of forming blister copper 45 from black copper or the like independently of the conversion of copper bearing sulphur compounds by a bessemerizing process which comprises initiating the conversion process by the use of extraneous heat, then continuing the process to a conclusion by utilizing the heat resulting from oxidation of metallic impurities in the black copper having a greater affinity for oxygen than copper, and thereafter repeating the process by re- 50 moving a portion only of the blister copper and retaining the balance as a heat reservoir to initiate the next cycle of the process.

In testimony whereof I have signed my name to this specification.

MARION H. MERRISS.